

## 1

3,557,013

PROCESS FOR SOLIDIFYING RADIOACTIVE  
WASTES BY ADDITION OF LIME TO PRE-  
CIPITATE FLUORIDE

Emile Detilleux, Werner Georg Hild, Gianfranco Lazaretto, Emilio Manuel Menchero-Lopez, and Rudolf Rometsch, all of Eurochemic, Mol, Belgium  
No Drawing. Filed Nov. 18, 1966, Ser. No. 595,325  
Claims priority, application Belgium, Apr. 7, 1966,  
26,521, Patent 679,231  
Int. Cl. G21c 19/46

U.S. Cl. 252—301.1

15 Claims

## ABSTRACT OF THE DISCLOSURE

A process for solidifying radioactive wastes containing at least one member selected from the group consisting of water-soluble fluoride, water-soluble sulphate and mixtures thereof comprising mixing with agitation at least one liquid radioactive waste with sufficient lime to neutralize the free sulphuric acid and to precipitate the free fluoride, evaporating the water present in the mixture until a hardenable paste is obtained, hardening the paste and enclosing the resulting block in a watertight covering.

The present invention concerns a process for the treatment of the decladding wastes, some medium level wastes and the high level wastes produced by plants reprocessing irradiated nuclear fuels.

The invention concerns a process for the insolubilisation and self-solidification of the effluents considered, after evaporation of the excess water. This process is simpler than those previously envisaged for the treatment of these particular effluents.

The object of the invention is to provide a process for the treatment, in the same operation, of the different types of solutions which constitute these categories of effluents—a process which has not been achieved before now.

The invention enables a solid compact mass to be obtained which lends itself particularly well to:

(a) Either being covered by a thin layer of an insoluble material such as bitumen,  
(b) Or being placed in drums or other leak-proof containers, where the level of radioactivity emitted by the solid mass would be incompatible with the radiation resistance of the covering material considered under (a).

This covering or containment acts as a barrier against leaching of the radioactive components contained in the solid mass. In particular, the covering of the solid considered under (a) makes it possible to avoid dispersing the radioactive solids in an inert mass which serves at the same time as binder and fixing agent preventing leaching. The process according to the invention also achieves a large volume reduction of the solids to be stored compared with that achieved by the known dispersion methods, proposed notably for slurries with specific activity inferior to that considered here, since in these known techniques the volume of active material incorporated in the inert mass represents only 40–50% of the total volume to be stored.

The process according to the invention does not require any operation at high temperature; this considerably reduces the risks of accelerated corrosion due to the

## 2

chemical nature of the solutions treated, as well as the risks of volatilising certain radioactive species. It is possible, therefore, to make use of the present-day construction materials and to avoid complex and delicate installations for the purification of gases and vapours produced by the operation. Because of this, the process according to the invention represents a notable simplification compared with other techniques which have been envisaged, such as calcination of the effluents or their incorporation in vitrified masses.

It is well known that nuclear fuels are essentially made up of a can of a weakly neutron-absorbing material, generally aluminium, magnesium, stainless steel or zirconium and its alloys such as "Zircaloy," and of an uranium core in the form of metal or oxide. After irradiation in a reactor, the core contains some plutonium and fission products in addition.

The technique of processing irradiated fuels is well known. The principal steps are as follows:

- 20 (1) Removal of the canning, either mechanically or chemically.
- (2) Dissolution of the core in nitric acid.
- (3) Separation of the uranium, plutonium and fission products by a series of extractions using selective agents such as tributyl phosphate.

Chemical decladding uses selective agents for dissolving the canning; these are caustic soda for aluminium, sulphuric acid for magnesium or stainless steel, and ammonium fluoride for zirconium or "Zircaloy." These decladding solutions constitute a very large part of the volume of medium level wastes produced by a reprocessing plant, as they contribute from 0.5 to 10 m<sup>3</sup> per ton of uranium treated. The activity contained in these solutions arises partly from the fission products which passed into the solution in the course of decladding, and partly from the activation of certain elements contained in the canning material. The activity level measured in these solutions can reach 10<sup>4</sup> Ci/m<sup>3</sup>, depending on the irradiation conditions and the cooling time of the fuel processed.

As an illustration, the average composition of the decladding solutions is given in the table hereafter:

|                  | Canning                                                | Average-composition      |
|------------------|--------------------------------------------------------|--------------------------|
| Aluminium:       |                                                        |                          |
| 45               | NaOH -----                                             | 2.5–3 M                  |
|                  | NaAlO <sub>2</sub> -----                               | <sup>1</sup> 1.5–3 M     |
| Magnesium:       |                                                        |                          |
|                  | H <sub>2</sub> SO <sub>4</sub> -----                   | 0.4–0.6 M                |
| 50               | MgSO <sub>4</sub> -----                                | <sup>2</sup> 1.25–1.75 M |
| Stainless steel: |                                                        |                          |
|                  | H <sub>2</sub> SO <sub>4</sub> -----                   | 2.8–3.2 M                |
|                  | (SS)SO <sub>4</sub> -----                              | <sup>3</sup> 0.8–1 M     |
| Zirconium:       |                                                        |                          |
|                  | NH <sub>4</sub> F -----                                | 0.5–0.6 M                |
| 55               | NH <sub>4</sub> NO <sub>3</sub> -----                  | 0.08–0.1 M               |
| Zircaloy:        |                                                        |                          |
|                  | (NH <sub>4</sub> ) <sub>2</sub> ZrF <sub>6</sub> ----- | <sup>4</sup> 0.55–0.65 M |

<sup>1</sup> 40–80 g./l. Al.

<sup>2</sup> 30–42 g./l. Mg.

<sup>3</sup> 45–55 g./l. SS.

<sup>4</sup> 50–58 g./l. Zr.

As no simple method for the treatment of these effluents has been proposed up to now, considerable research has been done into mechanical methods to take the place of chemical decladding. This research has led to complex, delicate and onerous techniques.

The other medium level wastes considered in the process according to the invention are produced essentially in the course of the third stage of reprocessing. They are made up of the concentrates resulting from the evaporation of different wastes of lower specific activity. Their composition is rather variable around the following values:

Main component:  $\text{NaNO}_3$ —100–400 g./l.

Traces of:  $\text{NO}_2^-$ ,  $\text{SO}_4^{2-}$ ,  $\text{CO}_3^{2-}$ ,  $\text{H}_3\text{PO}_4$ , U, other metals, Si, tributyl, dibutyl and monobutyl phosphates, kerosene.

Activity:  $10^6$ – $10^4$  Ci/m.<sup>3</sup>.

Quantity:  $\leq 5$  m.<sup>3</sup>/tonne U processed.

The large volumes of these types of waste, their relatively high radioactivity, their corrosive nature and their chemical composition which prevents their mixing, make prolonged liquid storage in separate tanks unacceptable from an economic point of view. Therefore, a treatment giving a drastic volume reduction and a transformation to a convenient form for prolonged, economic and safe storage is highly desirable.

The high level wastes are also produced during the third stage of the reprocessing. They contain essentially the bulk of the fission products as well as a certain number of other salts originating in the reagents added during processing and from corrosion of the equipment. At the end of the process, they are usually concentrated by evaporation. These high level wastes have variable compositions, which can be summarized as follows:

Fission and corrosion products:  $\leq 100$  g./l.<sup>1</sup>

Compounds originating in the reagents:  $\leq 120$  g./l.<sup>1</sup>

$\text{HNO}_3$ :  $\leq 11$  M

$\beta+\lambda$  activity:  $\leq 10^7$  Ci/m.<sup>3</sup>

Quantity:  $\leq 1$  m.<sup>3</sup>/t.

<sup>1</sup> Estimated as oxides.

Until now, no special treatment for the decladding waste has been proposed for resolving this problem in a simple manner. However, some treatment processes applied to very high level wastes (concentrated fission products, very low level wastes, and medium level wastes excluding decladding waste solutions are known or have been studied.

The most important of these known processes are:

- (a) various calcination processes,
- (b) incorporation in glass,
- (c) disposal in deep wells,
- (d) co-precipitation, flocculation, ion exchange, foam separation, etc.
- (e) incorporation in bitumen, cement, polymerising resins, paraffin, waxes, etc.

Although none of these methods has so far been adapted and used for decladding waste solutions, it is evident from the nature of the effluents and concentrates considered here that the application of the processes mentioned would lead to certain technical difficulties as well as very high costs.

Processes (a) and (b) present very serious technological and economic drawbacks due to the quantity of material to be treated; the salt content on the extremely corrosive nature of the solutions, the volatilisation of certain fission products, the operating temperatures and the risks of explosion involved.

Method (c) is applicable only in regions with a particular geological structure, and only a limited number of these exist.

The methods listed under (d) are uneconomic in view of the large volumes to be treated, and also because of the corrosion risks, content and variety of salts, which would necessitate the use of different processes appropriate to each case.

The techniques classed under (e) involve fire and explosion risks, as well as risks of radiation damage to the

sheathing material, and above all the volume reduction is insufficient.

The research carried out by the applicant into a method particularly suited to decladding wastes has led to surprising results which not only enable them to be solidified by a simple process but also enable other categories of radioactive wastes to be incorporated into the solid obtained.

The invention concerns a process for the solidification of radioactive wastes containing either water-soluble fluoride or a water-soluble mixture of fluoride and sulphate, possibly in the presence of a maximum of about 1 molar equivalent of nitrate for 3 molar equivalents of fluoride and/or sulphate. The process is characterized:

15 By the simultaneous mixing and agitation of at least one liquid effluent with lime, the quantity of lime used being at least equal to that necessary to neutralize the free sulphuric acid and/or to precipitate the free fluoride,

20 By the subsequent evaporation of the excess water present in the mixture until a slurry is formed which hardens on standing,

By the hardening of this slurry,

And by the sealing of the cake obtained in a watertight containment.

25 The first stage of the process according to the invention consists of precipitating the fluorides and sulphates from the decladding solutions with lime according to well known techniques. The normal treatment to apply would be the separation of the fluoride and sulphate precipitate,

30 by filtration for example. This would lead to a powdery product difficult to handle, from which the radioactive components could be easily leached. In addition, a large quantity of the radioactive substances would be left in the large volume of mother liquor, which would require a subsequent treatment.

It has now been found that if, instead of the separation of the precipitate by one of the usual methods (filtration, decantation, etc.), the bulk of the water is evaporated, a slurry results which contains 10 to 20% by

40 weight of water, is easy to handle and can be freely poured into any receptacle. On cooling and standing for several hours in air, the slurry hardens and enclose all the radioactive compounds.

The second and third stages of the process according to the invention therefore consist of distillation or evaporation of the water from the mixture until a paste containing 10 to 20% by weight of water is obtained, which is then allowed to harden to a dry cake.

The leachability of the cake obtained by this process 50 is then reduced to a very small amount (less than  $2.10^{-6}$  g./cm.<sup>2</sup> day) by covering the hard cake with an impermeable and insoluble material, which acts as a barrier between the cake containing the radioactive salts and the environment. This covering is the fourth step of the process according to the invention. An effective coating can be obtained by:

55 Immersing the dried cake successively into two baths of molten bitumen, one of low viscosity (170–190° C.), and the other of higher viscosity (130–150° C.).

Placing the dry block in a bitumen-lined container of metal or concrete, and completely filling the free space with molten bitumen. The previous coating of the internal walls may be omitted.

Covering materials other than bitumen, for example hardenable resins, cement, etc. can be considered.

60 In cases where the use of an impermeable, insoluble covering material would be incompatible with the level of radiation emitted by the block, the block can be placed in a leak-tight metal cask of corrosion resistant alloy. In this case, the risk of leaching the block by external agents is non-existent.

The principal advantage of the process according to the invention, apart from its simplicity and low cost, lies in the fact that the phenomenon of solidification of the concentrated slurry takes place over a large range of waste

compositions to be treated. This property is quite unforeseen, particularly for solutions with a low sulphate content. The mechanism of solidification of a slurry obtained by the process described in the present invention can very well be explained for solutions containing only sulphates, because it is similar to the solidification of plaster of paris, although the preparation of this is completely different.

The innovations of the present invention lie in the fact that it is not necessary to pass through a stage of forced drying as in the preparation of plaster of paris, and that it is possible, at the same time, to solidify fluoride solutions from the dissolution of zirconium and "Zircaloy," although it has been established that calcium fluoride crystallizes with no molecules of water of crystallization. In addition, the solidification process is not disturbed by the presence of soluble salts, such as  $MgSO_4$ ,  $NaNO_3$ , etc. This allows great latitude in the choice of volumes of solutions for solidification, as is shown, for example, by the following table:

|                        | Relative volumes |         |
|------------------------|------------------|---------|
|                        | Minimum          | Maximum |
| Al decladding solution | 0                | 1       |
| Mg decladding solution | 0                | 1       |
| SS decladding solution | 1                | 1       |
| Zr decladding solution | 2                | 5       |
| Concentrates           | 0                | 3       |
| High level waste       | 0                | 3       |

<sup>1</sup> Or 0.

<sup>2</sup> Or 1.

The incorporation and the solidification of the high level wastes is carried out either after neutralization of the free nitric acid by  $Ca(OH)_2$ ,  $CaO$ ,  $NaOH$ , etc. or after partial destruction of this acid by a reducing agent, such as sugar or formaldehyde, followed by neutralization of the remaining acid. This latter method leads to a reduction in volume to be treated.

This process according to the present invention can be applied to the final treatment and storage of radioactive waste solutions, and particularly to the treatment of de-cladding waste solutions, since the solid cakes obtained, suitably covered with an impermeable, insoluble material and placed in an appropriate containment, such as inexpensive casks, either can be stored in the open with no protection than an enclosure preventing entrance to the radiation zone, or can be thrown into the sea. In this case, the long-term storage costs are reduced to a minimum. For high level wastes, storage should probably be carried out for a certain period under shelter with forced ventilation to ensure the dissipation of the heat released by fission product decay.

Some ways of carrying out the process according to the invention are described in the following examples:

#### EXAMPLE 1

265 g. of lime (technical grade containing about 90%  $Ca(OH)_2$ ) are added in 15-20 minutes to 1.500 cm.<sup>3</sup> of "Zircaloy" decladding waste solution with a specific activity of 1 Ci/l. and mixed by a radial flow turbine type agitator. After distillation of 1.150 cm.<sup>3</sup> of water, the slurry obtained is cooled in a detachable cylindrical mould. A lifting hook is placed in the viscous mass, which is allowed to cool in air. After one hour, the paste has changed into a hard cake. After the cylindrical mould has been dismantled, the block is plunged, by means of the hook, into two successive baths of hot bitumen, the first at 180° C., the second at 130° C.

The coated block is then placed in a bath of distilled water kept between 21° C. and 30° C. for a period of 20 days, the water being renewed every 12 hours. The 80 litres of water used in this test are concentrated to 1 litre, and no activity is detected in the water.

The apparent density of the block, after it has been kept for 2 hours at 110° C. is 1.5 g./cm.<sup>3</sup> and the volume

reduction obtained (volume of initial solution/volume of block) is 3.3.

#### EXAMPLE 2

133 g. of technical grade lime are mixed in 10 to 20 minutes with 500 cm.<sup>3</sup> stainless steel decladding solution containing 3 M free  $H_2SO_4$  and 5 Ci radioactivity/l, in the way described in Example 1. 350 cm.<sup>3</sup> water are distilled and the resulting slurry treated as described in Example 1. The paste hardens in 45 minutes. No activity is detected in the water used for the leach tests. The apparent density of the block is 1.5 g./cm.<sup>3</sup>, and the volume reduction obtained is about 2.

#### EXAMPLE 3

500 cm.<sup>3</sup> sulphuric decladding solution identical to that of Example 2 are treated with 138 g. of technical grade lime in the way described in Example 1. After addition of the lime, 300 cm.<sup>3</sup> of an aluminum decladding solution with a specific activity of about 100 mCi/l. are also added. After evaporation of 540 cm.<sup>3</sup> of water, the paste, treated as in the preceding examples, hardens in 45 minutes. No activity is detected in the water used for leach tests. The apparent density of the block is 1.33 g./cm.<sup>3</sup>, with a corresponding volume reduction of 3.3.

#### EXAMPLE 4

500 cm.<sup>3</sup> magnesium decladding solution with a specific activity of 300 mCi/l. are treated with 46 g. of technical grade lime as in the previous examples. After evaporation of 425 cm.<sup>3</sup> of water, the paste hardens in 50 minutes. No activity is detected in the water used for leach tests on the block after it has been coated with bitumen. The apparent density of the block is 1.4 g./cm.<sup>3</sup>, and the corresponding reduction is 4.

#### EXAMPLE 5

500 cm.<sup>3</sup> magnesium decladding solution identical to that of Example 4, are treated with 26 g. technical grade lime. Then 468 cm.<sup>3</sup> aluminum decladding solution identical to that used in Example 3 are added. After evaporation of 700 cm.<sup>3</sup> water, the paste hardens in 75 minutes. No activity is detected in the water used for leach tests. The apparent density of the block is 1.2 g./cm.<sup>3</sup>, and the corresponding volume reduction is about 4.5.

#### EXAMPLE 6

250 cm.<sup>3</sup> stainless steel decladding solution (see Example 2) are mixed with 250 cm.<sup>3</sup> magnesium decladding solution (see Example 4), the neutralized with 80 g. technical grade lime. After evaporation of 350 cm.<sup>3</sup> water, the paste hardens in 1 hour. No activity is recorded in the leach test water. The apparent density of the block is 2.2 g./cm.<sup>3</sup>, and the volume reduction is 4.3.

#### EXAMPLE 7

250 cm.<sup>3</sup> stainless steel decladding solution (see Example 2) mixed with 250 cm.<sup>3</sup> decladding solution (see Example 4) are neutralized with 80 g. technical grade lime. Then 234 cm.<sup>3</sup> aluminum decladding solution (see Example 3) are added. After evaporation of 550 cm.<sup>3</sup> water, the paste hardens in 80 minutes. No activity is detected in the leach test water. The apparent density of the block is 2, and the corresponding volume reduction is 3.3.

#### EXAMPLE 8

350 cm.<sup>3</sup> stainless steel decladding solution (see Example 2), after neutralization with 80 g. technical grade lime, are mixed with 1.500 cm.<sup>3</sup> "Zircaloy" decladding solution (see Example 1). After evaporation of 1.570 cm.<sup>3</sup> water, the paste hardens in 80 minutes. The activity detected in the water from the leach tests corresponds to 10 p.p.m. of the total activity involved in the test. The apparent density of the block is 1.6 g./cm.<sup>3</sup>, and the volume reduction is 6.5.

7  
EXAMPLE 9

550 cm.<sup>3</sup> stainless steel decladding solution (see Example 2), after neutralization by 138 g. technical grade lime, are mixed with 300 cm.<sup>3</sup> aluminum decladding solution (see Example 3) and 1.500 cm.<sup>3</sup> "Zircaloy" decladding solution. After distillation of 2.000 cm.<sup>3</sup> water, the paste hardens in 90 minutes. The activity recorded in the water from the leach tests corresponds to 25 p.p.m. of the total activity involved in the test. The apparent density of the block is 2 g./cm.<sup>3</sup>, and the volume reduction is 7.4. 10

EXAMPLE 10

500 cm.<sup>3</sup> stainless steel decladding solution (see Example 2) mixed with 50 cm.<sup>3</sup> magnesium decladding solution (see Example 4) are neutralized with 125 g. technical grade lime. Then 50 cm.<sup>3</sup> aluminum decladding solution (see Example 3) and 1.500 cm.<sup>3</sup> "Zircaloy" decladding solution (see Example 1) are added. After evaporation of 1.735 cm.<sup>3</sup> water, the paste hardens in 90 minutes. The activity detected in the water from the leach tests corresponds to 20 p.p.m. of the total activity involved in the test. The apparent density of the block is 1.7 g./cm.<sup>3</sup>, and the volume reduction is 6. 15

EXAMPLE 11

250 cm.<sup>3</sup> stainless steel decladding solution (see Example 2) added to 50 cm.<sup>3</sup> magnesium decladding solution (see Example 4) are neutralized by 72 g. technical grade lime. After addition of 856 cm.<sup>3</sup> concentrate with a specific activity of 10 Ci/l. and 300 cm.<sup>3</sup> "Zircaloy" decladding solution (see Example 1), 1.100 cm.<sup>3</sup> water are distilled off. The paste hardens in 130 minutes. The activity detected in the water from the leach tests corresponds to 135 p.p.m. of the total activity involved in the test. The apparent density of the block is 2.1, and the volume reduction is 4.7. 20

EXAMPLE 12

250 cm.<sup>3</sup> stainless steel decladding solution (see Example 2), added to 50 cm.<sup>3</sup> magnesium decladding solution (see Example 4), are neutralized by 72 g. technical grade lime. After addition of 120 cm.<sup>3</sup> high level waste (100 ci/l.) previously partially neutralized by 43 g. technical grade lime and 300 cm.<sup>3</sup> "Zircaloy" decladding solution (see Example 1), 550 cm.<sup>3</sup> water are distilled off. The paste hardens in 20 minutes. The activity detected in the water from the leach tests corresponds to 85 p.p.m. of the total activity. The apparent density of the block is 1.8 g./cm.<sup>3</sup>, and the corresponding volume reduction is 3.3. 25

EXAMPLE 13

250 cm.<sup>3</sup> stainless steel decladding solution (see Example 2) and 50 cm.<sup>3</sup> magnesium decladding solution (see Example 4) are neutralized by 72 g. technical grade lime. After addition of 856 cm.<sup>3</sup> of concentrate (see Example 11) and 300 cm.<sup>3</sup> "Zircaloy" decladding solution (see Example 1), 120 cm.<sup>3</sup> high level waste are added (see Example 12), the acidity of which, previously reduced to 0.5 M HNO<sub>3</sub> by treatment with sugar, has been completely neutralized by 3 g. technical grade lime. After distillation of 1.250 cm.<sup>3</sup> water, the resulting paste hardens in 65 minutes. The activity detected in the water from the leach tests corresponds to 115 p.p.m. of the total. The apparent density of the block is 1.9, and the volume reduction is 4.6. 30

EXAMPLE 14

250 cm.<sup>3</sup> high level waste solution (see Example 13) mixed with 125 cm.<sup>3</sup> 12 M sulphuric acid are reduced by distillation to 250 cm.<sup>3</sup>. To this concentrate is added 250 cm.<sup>3</sup> stainless steel decladding solution (see Example 2) and the whole is neutralized by 176 g. technical grade lime. After addition of 300 cm.<sup>3</sup> "Zircaloy" decladding solution (see Example 1), 600 cm.<sup>3</sup> water are distilled off. The paste hardens in 35 minutes. The ac- 35

tivity detected in the leach test water corresponds to 120 p.p.m. of the total. The apparent density of the block is 2 g./cm.<sup>3</sup>, and the volume reduction is 4.9. 40

EXAMPLE 15

125 cm.<sup>3</sup> 12 M sulphuric acid are added to 500 cm.<sup>3</sup> high level waste solution (see Example 13). The mixture is evaporated down to a volume of 250 cm.<sup>3</sup>. Then 80 g. technical grade lime are added, 175 cm.<sup>3</sup> water are distilled off. The paste hardens in 30 minutes. The activity detected in the leach water corresponds to 150 p.p.m. of the total. The apparent density of the block is 1.7 g./cm.<sup>3</sup>, and the volume reduction is about 4. 45

What we claim is:

1. A process for solidifying radioactive wastes containing at least one member selected from the group consisting of water-soluble fluoride, water-soluble sulphate and mixtures thereof comprising mixing with agitation at least one liquid radioactive waste with sufficient lime to neutralize the free sulphuric acid and to precipitate the free fluoride, evaporating the water present in the mixture until a hardenable paste is obtained, hardening said paste and enclosing the resulting block in a water-tight covering. 50

2. A process according to claim 1, wherein sufficient water is evaporated to obtain a paste containing from about 10 to about 20% by weight of water. 55

3. A process according to claim 1 wherein the waste is obtained from the decladding of irradiated nuclear fuels. 60

4. A process according to claim 3, wherein a medium level waste is added to the decladding waste said medium level waste having an activity of from about 10<sup>2</sup> to 4 times 10<sup>3</sup> Ci/m.<sup>3</sup>. 65

5. A process according to claim 3, wherein to the decladding waste has been added a high level waste, the free acid contained therein having been neutralized beforehand, said high level waste having an activity of more than 3 times 10<sup>6</sup> Ci/m.<sup>3</sup>. 70

6. A process according to claim 1 wherein a high level waste is employed, the free acid contained therein having been neutralized beforehand, and to which fluoride and sulphate has been added before the addition of lime, said high level waste having an activity of more than 3 times 10<sup>6</sup> Ci/m.<sup>3</sup>. 75

7. A process according to claim 1, wherein the block is covered with an impermeable material, insoluble in water. 80

8. A process according to claim 7, wherein said impermeable material is selected from the group consisting of bitumens, asphalts, paraffins, and hardenable resins. 85

9. A process according to claim 1, wherein the paste is placed in a corrosion-resistant metal container after the water has been evaporated, allowed to harden, and the container is sealed with the hardened block inside. 90

10. A process according to claim 1 wherein said waste contains nitrate in a concentration of about 3 molar equivalents per molar equivalent of fluoride and sulphate. 95

11. A process according to claim 2, wherein the waste is obtained from the decladding of irradiated nuclear fuels. 100

12. A process according to claim 11, wherein medium level waste is added to the decladding waste, said medium level waste having an activity of from about 10<sup>2</sup> to about 4 times 10<sup>3</sup> Ci/m.<sup>3</sup>. 105

13. A process according to claim 11, wherein to the decladding waste has been added a high level waste, the free acid contained therein having been neutralized beforehand, said high level waste having an activity of at least 3 times 10<sup>6</sup> Ci/m.<sup>3</sup>. 110

14. A process according to claim 1, wherein said block is placed in a container. 115

15. A process according to claim 14, wherein said

block is first coated with an impermeable, insoluble material.

3,330,771 7/1967 Komatsv et al. ----- 252—301.1  
3,332,884 7/1967 Kelmar ----- 252—301.1

**References Cited****UNITED STATES PATENTS**

3,272,756 9/1966 Kaser ----- 252—301.1 5 F. M. GITTES, Assistant Examiner  
3,274,784 9/1966 Shock et al. ----- 252—301.1 X